# EUROPEAN PATENT SPECIFICATION

(11) **EP 3 409 829 B1**
(45) Date of publication and mention of the grant of the patent: **12.08.2020**
(21) Application number: 17173524.4
(22) Date of filing: 30.05.2017
(51) Int. Cl.: C10M 101/00, D06M 13/02, D01F 11/02, A24D 3/10

(54) **COMPOSITION COMPRISING HYDROCARBONS, EMULSIFIERS AND WATER, ITS USE AND PRODUCTS COMPRISING SUCH COMPOSITION**
ZUSAMMENSETZUNG MIT KOHLENWASSERSTOFFEN, EMULGATOREN UND WASSER, DEREN VERWENDUNG UND PRODUKTE MIT SOLCH EINER ZUSAMMENSETZUNG
COMPOSITION COMPRENANT DES HYDROCARBURES, DES ÉMULSIFIANTS ET DE L'EAU, SON UTILISATION ET PRODUITS COMPRENANT UNE TELLE COMPOSITION

(43) Date of publication of application: 05.12.2018
(73) Proprietor: Rhodia Acetow GmbH, 79108 Freiburg (DE)
(72) Inventor: SCHUTZ, Eckart, 79194 Gundelfingen (DE); MANN, Dieter, 79254 Oberried (DE)
(74) Representative: Trinks, Ole

(56) References cited:
- WO-A2-2006/007018
- US-A1- 2004 007 687
- JINJING LI ET AL: "Direct conversion of syngas into hydrocarbons over a core-shell Cr-Zn@SiO2@SAPO-34 catalyst", CHINESE JOURNAL OF CATALYSIS / DALIAN INSTITUTE OF CHEMICAL PHYSICS, vol. 36, no. 7, 1 July 2015 (2015-07-01), pages 1131-1135, XP055323548, AMSTERDAM, NL ISSN: 1872-2067, DOI: 10.1016/S1872-2067(14)60297-7

## Description

The present invention concerns composition comprising at least one hydrocarbon which is liquid at 20°C, obtained by a process of converting syngas into at least one hydrocarbon which is liquid at 20°C, at least one emulsifier and at least one aqueous phase. The invention further concerns a water in oil emulsion comprising the composition, a process in which they are applied to fibres or tow, fibres or tow comprising the composition and cigarette filters comprising such fibres or tow, wherein the fibres to tow are cellulose acetate fibres or tow.

It is known that in the production of various fibres and tows comprising fibres, auxiliary formulations are applied to the fibres and tows to avoid wear and rupture of the fibres, avoid electrostatic charging of fibres and reduce dust formation on fibres and roller points. Generally, these formulations comprise mineral oils, at least one emulsifier and water. Such formulations are described, for example, in WO2004007831.

It was now found that hydrocarbons which are liquid at 20°C, obtained by a process of converting syngas into at least one hydrocarbon which is liquid at 20°C, are suitable for being used in compositions that can be employed as auxiliary formulations in the manufacture of fibres and yarns. The compositions of the present invention often display several advantages, such as good lubricating properties, high viscosity index, low evaporation loss, stability of the composition, advantageous impurity profile and thus toxicology, stability against discoloration and staining, light stability, lower dust level in fibre production and, being manufactured from non-mineral hydrocarbon sources such as natural gas, are advantageous in view of environmental sustainability.

The invention thus concerns a composition comprising at least one hydrocarbon which is liquid at 20°C, obtained by a process of converting syngas into at least one hydrocarbon which is liquid at 20°C, at least one emulsifier and at least one aqueous phase, and a water in oil emulsion, comprising the composition. Another subject of the present invention is a process for making fibres or tow in which the composition or water in oil emulsion is applied to fibres or tow. Yet another object of the present invention is the use of the composition or water in oil emulsion in a manufacturing process as an auxiliary for the spinning of fibres, fibres or tow comprising the composition or water in oil emulsion and cigarette filters comprising such fibres or tow, wherein the fibres or the tow are cellulose acetate fibres or cellulose acetate tow.

In the present invention, designations in singular are in intended to include the plural; for example, "a solvent" is intended to denote also "more than one solvent" or "a plurality of solvents".

All "aspects" of the present invention are combinable.

In the context of the present invention, the term "comprising" is intended to include the meaning of "consisting of".

The composition according to the present invention can also be denoted as fibre finish, spinning finish or lubricant. The "at least one hydrocarbon which is liquid at 20°C, obtained by a process of converting syngas into at least one hydrocarbon which is liquid at 20°C" is a liquid hydrocarbon which is obtained by a catalysed process from syngas. Such processes often generally are described as Fischer-Tropsch-processes. In Fischer-Tropsch-processes, a mixture comprising carbon monoxide CO and hydrogen H₂, the so-called "syngas", is converted at elevated pressures, temperatures and in the presence of at least one catalyst, into a mixture of hydrocarbons. Desired chain lengths and isomerizations of the hydrocarbons can be steered by choosing the corresponding reaction conditions, such as temperature, pressure, syngas composition or presence of water. Syngas can be obtained by methods as gas to liquid (GTL) technology, wherein low molecular weight hydrocarbon materials, such as methane or natural gas mainly comprising methane, are converted into syngas. Other possible syngas sources are coal to liquid (CTL) process or biomass or biogas to liquid (BTL). According to the present invention, the at least one hydrocarbon that is obtained by a process of converting syngas is liquid at 20°C. The gaseous source that is the source for at least one hydrocarbon which is liquid at 20°C, obtained by a process of converting syngas into at least one hydrocarbon which is liquid at 20°C (and at ambient pressure of about 1 bar abs) and the manufacturing process clearly distinguishes the liquid hydrocarbon from mineral oils, as these hydrocarbons generally have a different structure and structure distribution and a different impurity profile, such as less sulphurous impurities, olefinic, aromatic and polycyclic aromatic impurities. The liquid hydrocarbons according to the present invention generally display a number of different characteristics, such as advantageous viscosity index and low evaporation losses. An advantageously high viscosity index indicates that the viscosity of the liquid hydrocarbon is relatively unaffected by temperature changes.

The composition according to the present invention comprises further at least one emulsifier. An emulsifier is generally defined as a surfactant which when present in small amounts facilitates the formation of an emulsion, or enhances its colloidal stability by decreasing either or both of the rates of aggregation and coalescence. In one aspect of the present invention, the at least one emulsifier is selected from the group consisting of sorbitan monoesters, derivatives of sorbitan monoesters, sorbitan diesters, derivatives of sorbitan diesters, sorbitan triesters, derivatives of sorbitan triesters, polyglycerol esters and derivatives of polyglycerol esters. It is preferred that the esters be esters with fatty acids. Generally, any fatty acid can be used as the fatty acid. Fatty acids denote aliphatic monocarboxylic acids derived from or contained in esterified form in an animal or vegetable fat, oil or wax. Natural fatty acids commonly have a chain of 4 to 28 carbons (usually unbranched and even-numbered), which may be saturated or unsaturated. Preferred fatty acids for esterification according to the present invention include stearic acid, oleic acid, lauric acid and ricinoleic acid ([R-(Z)]-12-hydroxy-9-octadecenoic acid). Alternatively, the fatty acids employed can be derived from maize, cotton oil, palm oil, groundnut oil, sesame oil, soy oil, safflower oil, copra, castor oil or other oils of native origin. The fatty acids can be hydrogenated or non-hydrogenated and condensed or noncondensed. Fatty acids with a carbon chain length of from 10 to 25 are preferred. Lauric acid is the most preferred fatty acid. In one aspect, sorbitan is ethoxylated before the esterification with one or more fatty acids. In another aspect, a sorbitanmonoester or a sorbitandiester or a sorbitantriester with one or more fatty acids is ethoxylated after the esterification with one or more fatty acids. Ethoxylation rates of from 5-30 mole ethylene oxide units per mole sorbitan are preferred. Ethoxylated sorbitanesters formed from sorbitanesters or sorbitanesters formed from ethoxylated sorbitan comprise derivatives of sorbitan monoesters, diesters and triesters. A preferred composition comprises sorbitan monolaurate and sorbitanmonolaurate ethoxylate as emulsifiers, wherein the sorbitanmonolaurate ethoxylate preferably has from 10 to 25, more preferably 18 to 22, and most preferably 20 repeat units of polyethylene glycol distributed across the different possible chains of the sorbitan scaffold. The preferred sorbitanmonolaurate ethoxylate is, for example, known as Polysorbate 20 (E432) or Tween®20. Other preferred emulsifiers are sorbitan monolaurate, sorbitan monooleate, sorbitan monopalmitate, polysorbate 80 (E433), polysorbate 65 (E436, polyoxyethene (20) sorbitan tristearate ), E471 (glyceryl monostearate, glyceryl distearate), E476 (Polyglycerol polyricinoleate), E477 (Propane-1,2-diol esters of fatty acids), E473 (Sucrose esters of fatty acids).

In one aspect of the present invention, the at least one emulsifier is present in the composition in an amount of from 15 wt% to 45 wt% of the composition. A content of from 20 to 40 wt% is preferred, and a content of from 25 to 35 wt% is most preferred. When more than one emulsifier is present in the composition, the foregoing amounts represents the combined amount of emulsifiers present in the composition.

A preferred emulsifier is an emulsifier mixture of sorbitan monolaurate and sorbitan monolaurate ethoxylate, wherein the sorbitan monolaurate ethoxylate preferably has from 10 to 25, more preferably 18 to 22, and most preferably 20 repeat units of polyethylene glycol distributed across the different possible chains of the sorbitan scaffold. The weight ratio of sorbitan monolaurate and sorbitan monolaurate ethoxylate generally is from 1:9 to 9:1, with the sum of both emulsifiers set at 10. Preferably, the weight ratio is from 3:7 to 7:3, and even more preferably of from 4:6 to 6:4. In a most preferred aspect, the ratio is from 5.1- 5.5 : 4.9 - 4.5.

In the composition according to the present invention, the composition comprises at least one aqueous phase. The at least one aqueous phase generally is present in an amount of from 0.1 to 15 wt%, preferably in an amount of from 3 to 10 wt%, and most preferably in an amount of from 5 to 7 wt%. This amount includes any aqueous phase contributed by other components, for example emulsifiers used for the composition. The aqueous phase preferably is water. Water includes de-mineralized water, de-ionized water, or otherwise appropriately filtered and treated water. In some cases, additives can be added to the aqueous phase.

The composition generally displays good lubricating properties, high viscosity index, low evaporation loss, stability of the composition, advantageous impurity profile and thus toxicology, stability against discoloration and staining, light stability, lower dust level in fibre production and, being manufactured from non-mineral hydrocarbon sources such as natural gas, are advantageous in view of environmental sustainability. Stability of the composition can be measured, for example, by controlling the turbidity of the composition. Light stability is also advantageous, as it is often undesirable to have discolorations of fibres.

According to the present invention, the at least one hydrocarbon which is liquid at 20°C generally has a viscosity of from 9 mm²/s at 40°C, which is approximately equal to 19 mm²/s at 20 °C, to 43 mm²/s at 40°C, which is approximately equal to 111 mm²/s at 20 °C. A viscosity of from 9.2 to 30 mm²/s at 40°C is preferred. The viscosity is determined according to ISO 3104.

In one aspect, the at least one hydrocarbon which is liquid at 20°C often has a carbon chain length distribution of from C18 to C50, preferably of from C20 to C29. The chain length distribution is measured by gas chromatography using an Agilent 6890 equipped with a capillary column HP-1 having an inner diameter of 0.25 mm and a film thickness of 0.1 µm and a FID detector using a temperature ramp from 60 °C to 320 °C at a heating rate of 25 °C per minute at a Helium flow rate of 1.1 ml per minute. A sample of 15 mg of the at least one hydrocarbon which is liquid at 20°C in 6 mL cyclohexane is measured, and the obtained spectrum compared to a spectrum of an external standard solution of n-alkanes (C16, C20, C26, C32 C38) in cyclohexane using the same experimental parameters the chain length distribution.

The composition according to the present invention preferably is used as lubricant or finish for spun fibres, in particular for fibres essentially consisting of cellulose acetate. The lubricant generally helps to reduce or prevent rupture of the fibres, electrostatic charging of fibres, dust formation on fibres, unwanted adhesion of fibres or elevated temperatures in processing. For the application of the lubricant to spun fibres, in particular to spun fibres essentially consisting of cellulose acetate, the composition according to the present invention generally is formulated into an oil in water emulsion comprising the composition. Generally, the oil in water comprises from 1 to 20 wt% of the composition according to the present invention and from 80 to 99% water. Preferably, the oil in water emulsion comprises from 1 to 10 wt% of the composition according to the present invention and from 90 to 99% water, and more preferably, the oil in water emulsion comprises from 1 to 5 wt% of the composition according to the present invention and from 95 to 99% water.

The composition according to the present invention can generally be obtained by mixing the ingredients under stirring, for example at room temperature. While the addition order often is not critical, it is preferred that the hydrocarbon is first provided, and that under continuous stirring, the other components are added in the order of emulsifiers, either combined or individually in case more than one emulsifier is present, and then aqueous phase, preferably water. It is often advantageous to stir the composition for approximately further 10 to 120 minutes. The procedure for the manufacture can be effected at room temperature of about 20°C, or at slightly elevated temperatures of up to 60°C.

The invention further concerns a manufacturing process which comprises a step of applying the composition according to the present invention, the water in oil emulsion according to the present invention or any other composition comprising the composition according to the present invention to fibres or tow comprising fibres. Preferably, the fibre is a cellulose acetate fibre or the tow is a cellulose acetate tow. In another aspect of the present invention, the invention concerns a manufacturing process which comprises the steps of
- providing a fibre dope
- spinning the fibre dope
- optionally drying or partially drying the spun fibres
- optionally forming a tow from the fibres
- applying the composition according to the present invention, the water in oil emulsion according to the present invention or any other composition comprising the composition according to the present invention to fibres or tow comprising fibres
- optionally drying the fibres or the tow
- optionally crimping the fibres or the tow
- optionally baling the fibres or the tow.

A fibre dope is a solution of fibre polymer, in particular cellulose acetate, in an appropriate solvent, which is in the case of cellulose acetate acetone. The fibres or the tow according to the manufacturing process are preferably cellulose acetate fibres or cellulose acetate tow. The dope can comprise further additives, such as degradation additives, colour additives or filtration additives. The cellulose acetate generally has a degree of substitution of from 1.5 to 3.0, preferably from 2.2 to 2.7. The degree of polymerisation generally is from 150 to 500, preferably from 180 to 280. The principles of spinning a dope of cellulose acetate are described, for example in P. Rustemeyer, Macromolecular Symposia, Volume 208, Issue 1, 2004, p. 267-292. A method for baling is described, for example, in WO2016/174162.

The invention concerns also fibres or a tow comprising the composition according to the present invention, or comprising the water in oil emulsion according to the present invention. The fibres or the tow are preferably cellulose acetate fibres or cellulose acetate tow. The fibres or tow generally have a LOF value (lubricant on fibre value) of from 0.1 to 3 wt%, preferably of from 0.7 to 2 wt%. The LOF value denotes and represents the lubricant less added water on either fibre or tow.

Another object of the present invention concerns the use of the composition according the present invention or the oil in water emulsion according to the present invention in a manufacturing process as an auxiliary for the spinning of fibres, in particular for spinning of cellulose acetate fibres.

A further object of the present invention is a cigarette filter, comprising the fibres or the tow according the present invention, which comprise the composition according to the present invention, or which comprise the water in oil emulsion according to the present invention, wherein the fibres or the tow are cellulose acetate fibres or cellulose acetate tow. The cigarette filter according to the present invention can have particularly advantageous properties in view of toxicological profile with regard to the hydrocarbons and their impurities and the low evaporation loss.

Should the disclosure of any patents, patent applications, and publications with the description of the present application to the extent that it may render a term unclear, the present description shall take precedence.

The following examples are intended to further explain the invention without limiting it.

All reagents can be obtained from commercial sources or manufactured from known procedures.

### Example 1

Shell Ondina X415 is provided at room temperature, and under continuous stirring, a mixture of sorbitan monolaurate (Alkamuls® S20) and sorbitan monolaurate ethoxylate (Tween®20) ratio 5.1 : 4.9 is added in an amount to equal 34 wt% of the total composition. Finally, de-ionized water is added under stirring to equal approximately 6 wt% of the total composition. The composition is stirred for a further 30 minutes. The composition is a stable, homogenous mixture.

### Example 2

The composition according to example 1 is added to de-ionized water under stirring at room temperature to equal 4 wt% of the final oil in water emulsion. The oil in water emulsion is stirred for another 60 minutes.

### Example 3

The oil in water emulsion is applied to cellulose acetate fibres after exit from the spinning cabinet, before entry into the crimper. The emulsion displays excellent lubricating qualities, and little dust formation is observed. A cigarette filter made from tow obtained from the spun cellulose acetate fibres displays an excellent low profile of impurities and low evaporation loss when submitted to standard tests.

## Claims

1. Composition comprising at least one hydrocarbon which is liquid at 20°C, obtained by a process of converting syngas into at least one hydrocarbon which is liquid at 20°C, at least one emulsifier and at least one aqueous phase.

2. Composition according to claim 1,
wherein the at least one emulsifier is selected from the group consisting of sorbitan monoesters, derivatives of sorbitan monoesters, sorbitan diesters, derivatives of sorbitan diesters, sorbitan triesters, derivatives of sorbitan triesters, polyglycerol esters and derivatives of polyglycerol esters.

3. Composition according to claim 1 or 2,
wherein the at least one emulsifier is present in an amount of from 15 wt % to 45 wt % of the composition.

4. Composition according to anyone of claims 1 to 3,
wherein the emulsifier is an emulsifier mixture of sorbitan monolaurate and sorbitan monolaurate ethoxylate.

5. Composition according to anyone of claims 1 to 4,
wherein the emulsifier mixture is a mixture of sorbitan monolaurate and sorbitan monolaurate ethoxylate, wherein the weight ratio of sorbitanmonolaurate to sorbitanmonolaurate ethoxylate is from 1:9 to 9:1.

6. Composition according to anyone of claims 1 to 5, at least one aqueous phase is present in an amount of from 0.1 to 15 wt %.

7. Composition according to anyone of claims 1 to 6,
wherein the at least one hydrocarbon which is liquid at 20°C has a viscosity of from 9 mm²/s at 40°C to 43 mm²/s at 40°C, when determined according to ISO 3104.

8. Composition according to anyone of claims 1 to 7,
wherein the at least one hydrocarbon which is liquid at 20°C has a carbon chain length distribution of from C18 to C50.

9. Water-in-oil emulsion, comprising the composition according to anyone of claims 1 to 8.

10. Manufacturing process which comprises a step of applying the composition according to anyone of claim 1 to 8, the water in oil emulsion of claim 9 or any other composition comprising the composition according to anyone of claim 1 to 7 to fibres or tow comprising fibres.

11. Process according to claim 10,
wherein the fibre is a cellulose acetate fibre or wherein the tow is a cellulose acetate tow.

12. Fibres or tow comprising the composition according to anyone of claim 1 to 8, or comprising the water in oil emulsion according to claim 9.

13. Fibres or tow according to claim 12,
wherein the LOF (lubricant on fibre) is from 0.1 to 3 wt%.

14. Use of the composition according to anyone of claims 1 to 8
or the oil in water emulsion according to claim 9 in a manufacturing process as an auxiliary for the spinning of fibres, in particular for spinning of cellulose acetate fibres.

15. Cigarette filter, comprising the fibres or the tow according to claim 12 or 13,
wherein the fibres or the tow are cellulose acetate fibres or cellulose acetate tow.

## Patentansprüche

1. Zusammensetzung, die mindestens einen bei 20°C flüssigen Kohlenwasserstoff, der durch ein Verfahren zur Umwandlung von Synthesegas in mindestens einen bei 20°C flüssigen Kohlenwasserstoff erhalten wird, mindestens einen Emulgator und mindestens eine wäßrige Phase enthält.

2. Zusammensetzung nach Anspruch 1,
wobei der mindestens eine Emulgator aus der Gruppe ausgewählt ist, die aus Sorbitanmonoestern, Derivaten von Sorbitanmonoestern, Sorbitandiestern, Derivaten von Sorbitandiestern, Sorbitantriestern, Derivaten von Sorbitantriestern, Polyglycerolestern und Derivaten von Polyglycerolestern besteht.

3. Zusammensetzung nach Anspruch 1 oder 2,
wobei der mindestens eine Emulgator in einer Menge von 15 Gew.-% bis 45 Gew.-% der Zusammensetzung vorhanden ist.

4. Zusammensetzung nach einem der Ansprüche 1 bis 3,
wobei der Emulgator eine Emulgatormischung aus Sorbitanmonolaurat und Sorbitanmonolaurat-ethoxylat ist.

5. Zusammensetzung nach einem der Ansprüche 1 bis 4,
wobei die Emulgatormischung eine Mischung aus Sorbitanmonolaurat und Sorbitanmonolaurat-Ethoxylat ist, wobei das Gewichtsverhältnis von Sorbitanmonolaurat zu Sorbitanmonolaurat-ethoxylat von 1:9 bis 9:1 beträgt.

6. Zusammensetzung nach einem der Ansprüche 1 bis 5, wobei mindestens eine wässrige Phase in einer Menge von 0,1 bis 15 Gew.-% vorhanden ist.

7. Zusammensetzung nach einem der Ansprüche 1 bis 6,
wobei der mindestens eine Kohlenwasserstoff, der bei 20°C flüssig ist, eine Viskosität von 9 mm²/s bei 40°C bis 43 mm²/s bei 40°C hat, wenn er gemäß ISO 3104 bestimmt wird.

8. Zusammensetzung nach einem der Ansprüche 1 bis 7,
wobei der mindestens eine Kohlenwasserstoff, der bei 20°C flüssig ist, eine Kohlenstoffkettenlängenverteilung von C18 bis C50 aufweist.

9. Wasser-in-öl-Emulsion, aufweisend die Zusammensetzung nach einem der Ansprüche 1 bis 8.

10. Herstellungsverfahren, das einen Schritt des Auftragens der Zusammensetzung nach einem der Ansprüche 1 bis 8, der Wasser-in-ÖI-Emulsion nach Anspruch 9 oder einer anderen Zusammensetzung, die die Zusammensetzung nach einem der Ansprüche 1 bis 7 umfasst, auf Fasern oder Tow, das Fasern umfasst, aufweist.

11. Verfahren nach Anspruch 10,
wobei die Faser eine Celluloseacetatfaser ist oder wobei das Tow ein Celluloseacetat-Tow ist.

12. Fasern oder Tow, aufweisend die Zusammensetzung nach einem der Ansprüche 1 bis 8 oder aufweisend die Wasser-in-ÖI-Emulsion nach Anspruch 9.

13. Fasern oder Tow nach Anspruch 12,
wobei das LOF (Schmiermittel auf der Faser) 0,1 bis 3 Gew.-% beträgt.

14. Verwendung der Zusammensetzung nach einem der Ansprüche 1 bis 8 oder der Öl-in-Wasser-Emulsion nach Anspruch 9 in einem Herstellungsverfahren als Hilfsmittel für das Spinnen von Fasern, insbesondere für das Spinnen von Celluloseacetat-Fasern.

15. Zigarettenfilter, aufweisend die Fasern oder das Tow nach Anspruch 12 oder 13,
wobei die Fasern oder das Tow Celluloseacetatfasern oder Celluloseacetat-Tow sind.

## Revendications

1. Composition comprenant au moins un hydrocarbure qui est liquide à 20°C, obtenu par un processus consistant à convertir un gaz de synthèse en au moins un hydrocarbure qui est liquide à 20°C, au moins un émulsifiant et au moins une phase aqueuse.

2. Composition selon la revendication 1,
dans lequel ledit au moins un émulsifiant est sélectionné parmi le groupe comprenant : monoesters de sorbitan, dérivés de monoesters de sorbitan, diesters de sorbitan, dérivés de diesters de sorbitan, triesters de sorbitan, dérivés de triesters de sorbitan, esters de polyglycérol et dérivés d'esters de polyglycérol.

3. Composition selon la revendication 1 ou 2,
dans lequel ledit au moins un émulsifiant est présent dans une quantité allant de 15 % en poids à 45 % en poids de la composition.

4. Composition selon l'une quelconque des revendications 1 à 3,
dans lequel émulsifiant est un mélange émulsifiant de monolaurate de sorbitan et de monolaurate éthoxylate de sorbitan.

5. Composition selon l'une quelconque des revendications 1 à 4, dans lequel le mélange émulsifiant est un mélange de monolaurate de sorbitan et de monolaurate éthoxylate de sorbitan, et dans lequel le rapport pondéral de monolaurate de sorbitan sur le monolaurate éthoxylate de sorbitan est de 1:9 à 9:1.

6. Composition selon l'une quelconque des revendications 1 à 5, dans lequel au moins une phase aqueuse est présente dans une quantité de 0,1 à 15 % en poids.

7. Composition selon l'une quelconque des revendications 1 à 6,
dans lequel ledit au moins un hydrocarbure qui est liquide à 20° C a une viscosité de 9 mm²/s à 40° C jusqu'à 43 mm²/s à 40° C, lorsqu'elle est déterminée en accord avec la norme ISO 3104.

8. Composition selon l'une quelconque des revendications 1 à 7,
dans lequel ledit au moins un hydrocarbure qui est liquide à 20° C présente une distribution de longueurs de chaîne carbone de C18 à C50.

9. Émulsion d'eau dans de l'huile, comprenant la composition selon l'une quelconque des revendications 1 à 8.

10. Procédé de fabrication qui comprend une étape consistant à appliquer la composition selon l'une quelconque des revendications 1 à 8, l'émulsion d'eau dans de l'huile selon la revendication 9, ou une quelconque autre composition comprenant la composition selon l'une quelconque des revendications 1 à 8 à des fibres ou à des mèches comprenant des fibres.

11. Procédé selon la revendication 10,
dans lequel la fibre est une fibre d'acétate de cellulose, ou dans lequel la mèche est une mèche d'acétate de cellulose.

12. Fibres ou mèche comprenant la composition selon l'une quelconque des revendications 1 à 8, ou comprenant l'émulsion d'eau dans de l'huile selon la revendication 9.

13. Fibres ou mèche selon la revendication 12, dans lequel la quantité "LOF" (lubrifiant sur fibres) est de 0,1 à 3 % en poids.

14. Utilisation de la composition selon l'une quelconque des revendications 1 à 8, ou de l'émulsion d'huile dans de l'eau selon la revendication 9 dans un processus de fabrication à titre d'auxiliaire pour le filage de fibres, en particulier pour le filage de fibres d'acétate de cellulose.

15. Filtre de cigarette, comprenant les fibres ou la mèche selon la revendication 12 ou 13, dans lequel les fibres ou la mèche sont des fibres d'acétate de cellulose ou une mèche d'acétate de cellulose.
